

## UNITED STATES PATENT OFFICE.

WILLIS EUGENE RAGAN, OF ATLANTA, GEORGIA.

## METHOD OF PROTECTION AGAINST ATTACK BY MITES OR INSECTS.

No Drawing.

Application filed April 4, 1925. Serial No. 20,859.

This invention is an improvement in a method of protecting persons from attack by the red bug or chigger. This mite, technically known as *Trombiculoides holosericeum*, infests woodlands, and being caught up on the clothing of a person brushing against the bushes which harbor it, finds its way to the skin of its host where it causes an itching lesion by burrowing into the skin.

10 The principal object of the invention is to afford protection to the person against attack by the mite, by impregnating the outer wearing apparel with an insecticide in powdered form, preferably sulphur.

15 My invention is carried out by sprinkling sulphur or powder over the outer clothing, and then subjecting the clothing to a temperature of about 125° C. either in a dry oven having a thermostatic control, or by means of 20 steam under pressure. The heat converts the sulphur powder into a thin liquid which is absorbed by the fabric of the garment, permeating the pores thereof, whereupon the garment is removed from the influence of the 25 heat. Upon cooling, the absorbed liquid reverts to a powder, but this powder is more finely divided than before and is so immeshed in the pores of the clothing that it will remain indefinitely and not be brushed off by 30 the bushes harboring the red bug, as is the case if the powder is merely dusted on.

I have found that my method is exceedingly efficacious in preventing attack by this mite, and that no uncomfortable or injurious 35 effects are experienced by a person wearing garments thus treated.

The foregoing description has been given for purposes of illustration, and no undue 40 limitations should be deduced therefrom, but the appended claims should be construed as broadly as permissible, in view of the prior art.

Having thus described my invention what I claim is:—

1. The method of treating a garment for the purpose of protecting a person wearing such garment against attack by the red bug, consisting in powdering a protective garment of a person with sulphur, subjecting the powdered garment to a temperature of about 125° 50 C. to thereby convert the powder to a thin liquid, allowing such liquid to be absorbed by the garment, then cooling the garment to thereby convert the absorbed liquid to a powder. 55

2. The method of treating a garment for the purpose of protecting a person wearing such garment against attack by mites and insects, consisting of powdering a protective garment with sulphur, subjecting such powdered garment to heat sufficient to convert the sulphur powder to a liquid, allowing such liquid to be absorbed by the garment, then allowing the garment to cool and thereby convert the absorbed liquid to a powder. 60

3. The method of treating a fabric to render it obnoxious to mites and insects, consisting in powdering the fabric with sulphur, subjecting the powdered fabric to sufficient heat to convert the sulphur to a thin liquid 70 to thereby allow the liquid to permeate the pores of the fabric, and thereafter allowing the fabric to cool to thereby convert the liquid to a fine powder. 65

4. The method of treating a garment to 75 protect a person wearing the same against attack by mites and insects, consisting in impregnating the pores of the garment with liquid sulphur by subjecting the garment with sulphur powdered thereon to heat, and then converting the liquid sulphur to a powder. 80

In testimony whereof I hereunto affix my signature.

WILLIS EUGENE RAGAN.